# EUROPEAN PATENT SPECIFICATION

(11) **EP 2 113 021 B1**
(45) Date of publication and mention of the grant of the patent: **12.06.2019**
(21) Application number: 08709441.3
(22) Date of filing: 18.02.2008
(51) Int. Cl.: C10M 101/02, C10M 107/00, C10M 107/10, C10N 30/04, C10N 30/10, C10N 40/25

(54) **METHOD FOR MAKING A LUBRICANT BASE OIL AND ITS USE**
VERFAHREN ZUR HERSTELLUNG VON BASISÖL UND IHR VERWENDUNG
PROCÉDÉ POUR LA PREPARATION D'UN HUILE DE BASE ET SON UTILISATION

(30) Priority: 21.02.2007 EP 07250739
(43) Date of publication of application: 04.11.2009
(73) Proprietor: BP p.l.c., London SW1Y 4PD (GB)
(72) Inventor: AMES, Stephen, Bruce, Pepper Pike, Ohio 44124 (US); DAVIES, John, Philip, Berkshire RG8 7RP (GB); LIDDY, John, Philip, Middlesex TW18 3JA (GB); LIM, Kok-Chye, Chelshire CW6 0PY (GB)
(74) Representative: Hill, Simon Stephen
(86) International application number: PCT/GB2008/000554
(87) International publication number: WO 2008/102114

(56) References cited:
- EP-A- 0 709 447
- EP-A1- 0 475 560
- EP-A1- 1 803 799
- EP-A2- 0 839 891
- DE-A1- 2 656 652
- GB-A- 1 027 518
- GB-A- 1 237 291
- GB-A- 1 237 292
- GB-A- 1 572 794
- GB-A- 2 083 494
- US-A- 4 777 307
- US-A- 5 602 086
- US-A- 5 911 874
- US-A1- 2003 100 453
- G Van Der Waal: "Improving the Performance of Synthetic Base Fluids with Additives", , 1 December 1987 (1987-12-01), XP055423181, Retrieved from the Internet: URL:http://onlinelibrary.wiley.com/store/1 0.1002/jsl.3000040402/asset/3000040402_ftp .pdf?v=1&t=j9qxe1dc&s=b9b23ae00c6caef127d0 5f31ec61b99fe52e6b5c [retrieved on 2017-11-09]
- P Mcshane ET AL: "Title: Coking Tendency of Dielectric Fluids at Contact Surfaces - Phase I: Constant Current", , 15 May 2003 (2003-05-15), XP055423021, Retrieved from the Internet: URL:http://www.spxtransformersolutions.com /assets/documents/41CokingStudy.pdf [retrieved on 2017-11-08]

## Description

This invention relates to lubricant base oils and lubricant compositions and to methods for making them.

Lubricant compositions generally comprise a base oil and one or more additives. According to API standard 1509, "ENGINE OIL LICENSING AND CERTIFICATION SYSTEM", November 2004 version 15th edition Appendix E, base stocks which are used for base oils are defined as belonging to one of five Groups as set out in Table I below.

**Table I**

| Group | Saturated hydrocarbon content (wt%) | | Sulphur content (wt%) | | Viscosity Index |
|---|---|---|---|---|---|
| I | < 90 | and/or | > 0.03 | and | ≥ 80 and < 120 |
| II | ≥ 90 | and | ≤ 0.03 | and | ≥ 80 and < 120 |
| III | ≥ 90 | and | ≤ 0.03 | and | ≥ 120 |
| IV | polyalpha olefins | | | | |
| V | all base stocks not in Groups I, II, III or IV | | | | |

Group I base stocks are generally preferred to Group II base stocks for the manufacture of lubricant compositions for marine 2-stroke and 4-stroke engines, particularly for engines operating on heavy fuel oil. However, Group II base stocks are becoming increasingly more readily available because older manufacturing capacity for Group I basestock is being closed and new manufacturing capacity tends to manufacture Group II base stock.

Group II base stocks may have some performance disadvantages compared to Group I base stocks when used in some lubricant compositions, for example in marine lubricants. These disadvantages may include poorer dispersancy, poorer seal swell performance, poorer solubility of additives, lower compatibility with fuel oil in marine engine applications (which can lead to deposit formation, for example in cool parts of the engine) and/or in some aspects, poorer oxidative stability.

Hydroprocessed base stocks may have advantages and disadvantages (Deckman, D.E. et al., Hart's Lubricants World, July 1997, pages 46 - 50) when used in industrial lubricant applications (Deckman D. E. et al., Hart's Lubricants World, Sept 1997, pages 20-26) and in commercial, personal vehicle and marine engine oils (Deckman D. E. et al., Hart's Lubricants World, Sept 1997, pages 27 - 28).

According to Deckman D. E. et al., in Hart's Lubricants World, Sept 1997, pages 27 - 28, "*Because hydrocracking results in a viscosity loss of the base stocks, marine oils cannot generally be formulated solely with hydrocracked base stocks, but require the use of significant amounts of bright stock. However, the use of bright stock is not desirable because of the presence of oxidatively unstable aromatics*"*.*

Base stocks which are made by hydroprocessing, including Group II and Group III base stocks, have lower aromatics content and lower sulphur content than Group I base stocks. GB2083494, US4777307, EP0709447, US2003/100453, GB1237291, GB1237292 and DE2656652 relate to hydroprocessed oils. They disclose the addition of either aromatic extracts, aromatic fractions, multiring aromatic compounds or bright stock to these for improving their oxidation stability. EP0839891 discloses aromatic process oils for rubber extenders having polycyclic aromatics content less than 3 %.

Base stocks derived from Fischer-Tropsch synthesised, waxy, paraffinic hydrocarbon materials also have a low aromatics content and so may also exhibit at least some of the poorer performance of Group II and Group III base stocks compared to Group I base stocks. WO 00/14187 and WO 2005/066314 relate to lubricant compositions comprising Fischer Tropsch derived base stock.

There remains a need for a base oil composition which overcomes, or at least mitigates these problems.

It has now been found that the use of 0.2 to 30 % by weight of an aromatic extract in a base oil comprising base stock, which base stock comprises at least 95 % by weight saturated hydrocarbons, can overcome or at least mitigate these problems.

Thus, according to one aspect of the present invention, there is provided method of making a liquid marine lubricant base oil composition which method comprises blending: (i) a base stock comprising at least 95 % by weight saturated hydrocarbons, the base stockcomprising a hydroprocessed base stock and/or a base stock derived from Fischer-Tropsch synthesised, waxy, paraffinic hydrocarbon material, with (ii) 0.2 to 30 % by weight of an aromatic extract which has an aromatics content of 60 to 85% by weight as measured by ASTM D 2007 and a dimethyl sulphoxide extractable polycyclic aromatics content of less than 3 weight % as measured by IP 346, to make a liquid lubricant base oil composition.

The present invention solves the problem defined above by the use of 0.2 to 30 % by weight of an aromatic extract which has a dimethyl sulphoxide extractable polycyclic aromatics content of less than 3 weight % in a liquid lubricant base oil composition which base oil comprises a base stock comprising at least 95 % by weight saturated hydrocarbons. This provides a lubricant base oil which overcomes or at least mitigates, at least some of the deficiencies which may be associated with such base stocks.

The lubricant base oil composition prepared according to the method of the present invention comprises 0.2 to 30 % by weight of an aromatic extract. Preferably, the lubricant base oil composition comprises 0.2 to 18 % or 1.0 to 30 % by weight of the aromatic extract. More preferably, the lubricant base oil composition comprises 1.0 to 18 % by weight aromatic extract.

Preferably, the base stock comprising at least 95 % by weight saturated hydrocarbons comprises a hydroprocessed base stock and/or a base stock derived from Fischer-Tropsch synthesised, waxy, paraffinic hydrocarbon material. The lubricant base oil composition prepared according to the method of the present invention overcomes or at least mitigates, at least one of the deficiencies which may be associated with such base stocks, for example those deficiencies selected from the group consisting of poor dispersancy (for example, of soot and/or deposits), poor seal swell performance, poor solubility of additives and low compatibility with fuel oil in marine engine applications (which can lead to deposit formation, for example in cool parts of the engine), and also in some aspects, poor oxidative stability.

Thus, according to a further aspect of the present invention there is provided the use of 0.2 to 30 % by weight of an aromatic extract which has an aromatics content of 60 to 85 % by weight as measured by ASTM D 2007 and a dimethyl sulphoxide extractable polycyclic aromatics content of less than 3 weight % as measured by IP 346 in a liquid marine lubricant base oil composition which base oil comprises a base stock comprising at least 95 % by weight saturated hydrocarbons, which hydrocarbons comprise a hydroprocessed base stock and/or a base stock derived from Fischer-Tropsch synthesised, waxy, paraffinic hydrocarbon material, to mitigate at least one of the deficiencies of the base stock selected from the group consisting of poor dispersancy, poor seal swell performance, poor solubility of additives and low compatibility with fuel oil in marine engine applications.

In particular, the present invention provides a method which uses a defined amount of aromatic extract, to make a base oil using a hydroprocessed base stock which may comprise for example, a Group II base stock and/or a Group III base stock, and/or using a base stock which may comprise a polyalphaolefin and/or using a base stock derived from Fischer-Tropsch synthesised, waxy, paraffinic hydrocarbon material. This base oil can be used in applications where a Group I base stock has conventionally been used, such as for example, in marine engine applications, for example in 2-stroke marine diesel engine cylinder oils, 2-stroke marine diesel engine system oils and 4-stroke marine diesel engine crankcase lubricant compositions.

The aromatic extract is preferably made by the treatment of at least one refinery process stream in a solvent extraction process. Suitable solvent extraction process include contacting the at least one refinery process stream with a solvent such as furfural, n-methylpyrrolidone, sulphur dioxide, Duo-Sol™ or phenol to selectively extract from the refinery stream, aromatic and heterocyclic materials and to form a solution of these materials in the solvent. The solvent is then recovered from the solution for recycle to the extraction process; the resultant product being the aromatic extract.

The manufacture of aromatic extracts is known in the art and is described for example in *"*Lubricant base oil and wax processing" A. Sequeira, pages 81-118, pub. Marcel Dekker Inc. New York, 1994.

The aromatic extract may be a residual aromatic extract, which may be made by treatment in an extraction process, of solvent deasphalted vacuum residue (also known as DAO) made using Duo-Sol™, propane, butane or mixtures thereof as the solvent for the deasphalting.

The aromatic extract may be a distillate aromatic extract (DAE) which is an aromatic extract made by treatment in an extraction process, of a distillate stream from a vacuum distillation process. Preferably, the distillate aromatic extract is a treated distillate aromatic extract which is a distillate aromatic extract which has been subjected to at least one further treatment. Suitably, the at least one further treatment is selected from the group consisting of hydrotreatment, hydrogenation, hydrodesulphurisation, clay treatment, acid treatment and further solvent extraction.

The aromatic extract has an aromatics content of 60 to 85 weight %, which is measured by ASTM D 2007.

The aromatic extract may have properties such as those described in Concawe Product Dossier 92/101 "Aromatic Extracts".

The distillate aromatic extract may have a boiling point in the range 250 - 680 °C, which may be measured according to ASTM D 2887. The distillate aromatic extract may have a kinematic viscosity at 40 °C in the range 5 - 18000 mm²/s, which may be measured according to ASTM D 445. The distillate aromatic extract may have a kinematic viscosity at 100 °C in the range 3-60 mm²/s, which may be measured according to ASTM D 445. The distillate aromatic extract may have an average molecular mass in the range 300 - 580, which may be measured according to ASTM D 2887. The distillate aromatic extract may have a carbon number range in the range C₁₅ - C₅₄, which may be measured according to ASTM D 2887. The distillate aromatic extract has an aromatic content in the range 65 - 85 weight %, which may be measured according to ASTM D 2007.

The residual aromatic extract may have a boiling point of greater than 380 °C, which may be measured according to ASTM D 2887. The residual aromatic extract may have a kinematic viscosity at 40 °C of greater than 4000 mm²/s, which may be measured according to ASTM D 445. The residual aromatic extract may have a kinematic viscosity at 100 °C in the range 60 - 330 mm²/s, which may be measured according to ASTM D 445. The residual aromatic extract may have an average molecular mass of greater than 400, which may be measured according to ASTM D 2887. The residual aromatic extract may have a carbon number range of greater than C₂₅, which may be measured according to ASTM D 2887. The residual aromatic extract has an aromatic content in the range 60 - 85 weight %, which may be measured according to ASTM D 2007.

Aromatic extracts may comprise polycyclic aromatic compounds (PAC's) some of which are carcinogens. The amount of material (weight %) which can be extracted into dimethyl sulphoxide (DMSO) is used as an indication of the amount of unacceptable material (including polycyclic aromatic compounds) in the aromatic extracts. IP 346 (Institute of Petroleum Test Method 346) is the method used for determining weight % DMSO extract according to the present invention. Aromatic extracts with greater that 3 weight % dimethyl sulphoxide extractable polycyclic aromatics content are classed as carcinogenic and give rise to requirements in several jurisdictions that the material be labelled with certain symbols and risk phrases to identify health, safety and environmental hazards. For this reason at least, the aromatic extract has less than 3 weight % dimethyl sulphoxide extractable polycyclic aromatics content (low PCA extract). More preferably, the aromatic extract is a residual aromatic extract or a treated distillate aromatic extract, with less than 3 weight % dimethyl sulphoxide extractable polycyclic aromatics content.

Preferably, the aromatic extract does not contain any significant amount of wax, because if present, wax may deposit in use.

The base stock used in the present invention comprising at least 95 % by weight saturated hydrocarbons may comprise both a hydroprocessed base stock and a base stock derived from Fischer-Tropsch synthesised, waxy, paraffinic hydrocarbon material. Suitably, base stock used in the present invention comprising at least 95 % by weight saturated hydrocarbons may comprise a hydroprocessed base stock or a base stock derived from Fischer-Tropsch synthesised, waxy, paraffinic hydrocarbon material.

The hydroprocessed base stock is preferably a Group II and/or Group III base stock, such as defined according to API standard 1509, "ENGINE OIL LICENSING AND CERTIFICATION SYSTEM", November 2004 version 15th edition Appendix E.

The base stock comprising at least 95 % by weight saturated hydrocarbons preferably comprises a Group II and/or Group III base stock, such as defined according to API standard 1509, "ENGINE OIL LICENSING AND CERTIFICATION SYSTEM", November 2004 version 15th edition Appendix E, comprising at least 95% by weight saturated hydrocarbons.

Preferably, the Group II base stock or Group III base stock is a hydroprocessed base stock which may be made by hydroprocessing, preferably of vacuum distillate or deasphalted vacuum residue, or by hydroisomerising the bottoms stream from a clean fuels hydrocracker. The manufacture of base stock by hydroprocessing is known in the art and is described for example in "Lubricant base oil and wax processing" A. Sequeira, pages 119 - 152, pub. Marcel Dekker Inc. New York, 1994.

The base stock comprising at least 95 % by weight saturated hydrocarbons may comprise one or more polyalphaolefin.

The base stock derived from a Fischer-Tropsch synthesised, waxy, paraffinic hydrocarbon material may be made by any suitable known process for the manufacture of base stock from Fischer Tropsch process. Processes for the manufacture of a base stock derived from Fischer-Tropsch synthesised, waxy, paraffinic hydrocarbon material which may be used, are described for example in US4943672, EP-A-0668342 and EP-A-0776959. Thus, the base stock may be made by the steps of (i) producing Syngas, (ii) Fischer-Tropsch synthesis of hydrocarbons from the Syngas, (iii) hydrocracking of the hydrocarbons to produce naphtha and diesel/kerosene fuel process streams together with a waxy paraffinic residue and (iv) hydroisomerising the waxy residue to produce the base stock.

The liquid lubricant base oil composition is prepared according to the method of the present invention by blending a base stock comprising at least 95 % by weight saturated hydrocarbons with sufficient an aromatic extract to make the lubricant base oil composition. The blending may be performed in a batch blending process or in a continuous blending process. Batch blending may be performed by introducing the base stock and aromatic extract into a blend kettle whilst stirring and/or agitating the blending components. Continuous blending may be performed using an in-line mixer to blend the base stock and aromatic extract. Heating may be necessary during the blending to facilitate handling of the aromatics extracts.

Preferably, the liquid lubricant base oil composition prepared according to the method of the present invention has a viscosity in the range 7 to 40 cSt at 100° C.

The liquid lubricant base oil composition is particularly useful for the manufacture of 2-stroke marine diesel engine cylinder oils, 2-stroke marine diesel engine system oils or 4-stroke marine diesel engine crankcase lubricant compositions.

The liquid lubricant composition prepared according to the method of the present invention comprises a liquid lubricant base oil composition as herein defined and may comprise one or more additives, preferably selected from the group consisting of detergents, dispersants, anti-wear additives, anti-oxidants, anti-foams, corrosion inhibitors, pour point depressants, friction modifiers, tackifiers and viscosity index improvers.

The concentrations of additives in the lubricant composition depend upon the use for which the lubricant composition is intended. One or more anti-oxidants may be present in the lubricant composition at a total concentration by weight of 0 to 1 %, usually at a concentration by weight of not greater than 0.5 %.

One or more anti-wear additives may be present in the lubricant composition at a total concentration by weight of 0 to 2 %, usually at a concentration by weight of not greater than 1 %.

One or more high over-based detergents may be present in the lubricant composition at a total concentration by weight of 0 to 40 %.

One or more low base detergents may be present in the lubricant composition at a total concentration by weight of 0 to 10 %.

One or more neutral detergents may be present in the lubricant composition at a total concentration by weight of 0 to 2 %.

One or more dispersants may be present in the lubricant composition at a total concentration by weight of 0 to 10%.

One or more anti-foams may be present in the lubricant composition at a total concentration by weight of 0 to 0.1 %.

One or more corrosion inhibitors may be present in the lubricant composition at a total concentration by weight of 0 to 1 %.

One or more pour point depressants may be present in the lubricant composition at a total concentration by weight of 0 to 1 %.

One or more friction modifiers may be present in the lubricant composition at a total concentration by weight of 0 to 5%.

One or more tackifiers may be present in the lubricant composition at a total concentration by weight of 0 to 15 %.

One or more viscosity index improvers may be present in the lubricant composition at a total concentration by weight of 0 to 20 %.

The concentration ranges for the additives may be independent of each other. Alternatively, combinations of such concentration ranges may be used for any particular lubricant composition.

The liquid lubricant compositions prepared according to the method of the present invention may be used as a 2-stroke marine diesel engine cylinder oil, 2-stroke marine diesel engine system oil or 4-stroke marine diesel engine crankcase lubricant composition.

The concentration ranges for additives for such lubricant compositions are given in the Table II below. Such concentration ranges may be independent of each other. Alternatively, combinations of such concentration ranges may be used for any particular lubricant composition.

**Table II.**

| Concentration ranges are expressed in % by weight of the liquid lubricant composition. | | | | | | | | | | |
|---|---|---|---|---|---|---|---|---|---|---|
| Lubricant Composition | High overbased detergent | Low base detergent | Anti-wear additive | Neutral detergent | Dispersant | Anti-foam | Corrosion inhibitor | Pour Point Depressant | Viscosity Index Improver | Anti-oxidant |
| Cylinder oil lubricant | 5 - 40 | 0 - 10 | 0 - 2 | 0 - 2 | 0 - 4, preferably 0.5 - 4 | 0 - 0.1 | 0 - 1 | 0 - 1 | 0 - 20 | 0 - 1 |
| 2-stroke crank case lubricant (System Oil) | 0 - 5 | 0 - 5 | 0 - 1 | 0 - 2 | 0 - 1.5 | 0 - 0.1 | 0 - 0.2 | 0 - 1 | 0 - 20 | 0 - 1 |
| 4-stroke crank case lubricant | 3 - 30 | 0 - 10 | 0 - 2 | 0 - 2 | 0 - 10, preferably 0.3 - 10 | 0 - 0.1 | 0 - 0.2 | 0 - 1 | 0 - 20 | 0 - 1 |

The invention will now be described by way of example only and with reference to Figure 1 which is a graph of the performance of base oil with various amounts of aromatic extract.

In these experiments a hydroprocessed base stock was a Group II base stock comprising at least 97 % by weight saturated hydrocarbons was used. The aromatic extract was a low PCA brightstock extract (less than 3 % polycyclic aromatics, brightstock furfural extract) provided by Shell. Properties of these components are given in Table III below.

**Table III General properties of components**

| Components | Test Method | Jurong 500N Base stock | Aromatic Extract (AE) |
|---|---|---|---|
| Type | | Group II | Aromatic Extract |
| KV40, mm²/s (cSt) | IP71 | 91.58 | - |
| KV100, mm²/s (cSt) | IP71 | 10.64 | 71.47 |
| VI | IP226 | 99 | - |
| Density, g/cm (15 °C) | IP365 | 0.8746 | 0.9897 |
| Flash point (PMCC), °C | IP34 | 232.3 | 284.3 |
| Flash point (COC), °C | IP36 | 266 | 308 |
| Pour point, °C | IP15 | -18 | -12 |
| Colour | ASTM D1500 | 0.1 | >8 |
| TAN, mg KOH/g | IP1A | <0.05 | 0.09 |
| TBN, mg KOH/g | IP276 | <0.05 | 2.14 |
| Sulphur, % | ASTM D4951 | 0.0037 | 4.13 |
| Nitrogen, % | ASTM D5762 | 0.0027 | 0.11 |
| Demulsibility, secs | IP19 | 75 | - |
| Dialysis, % wt | BAM72 | <0.1 | <0.1 |
| Oxidation IP48 | IP48 | | Rams bottom carbon - 4.3% |
| Viscosity ratio | | 3.06 | |
| Carbon before, wt. % | | 0.05 | |
| Carbon after, wt. % | | 0.60 | |
| Carbon, Δ | | 0.55 | |
| Carbon types wt % | BAM76 | | Viscosity too high to permit determination |
| Carbon, aromatic C_{A} | | 1.2 | |
| Carbon, naphthenic C_{N} | | 67.2 | |
| Carbon, paraffinic C_{P} | | 31.6 | |
| Hydrocarbon types wt % | D2007 | | |
| Saturates | | 97.9 | 11.3 |
| Aromatics | | 2.1 | 80.2 |
| Polars | | <0.1 | 8.5 |

The base stock and aromatic extract were shown not to contain any significant amounts of waxy materials. Base oil compositions were prepared by blending the aromatic extract (AE) with various amounts of the Group II base stock. Properties of the base oil compositions are given in Table IV below.

**Table IV**

| Sample | Test Method | Example 1 | Example 2 |
|---|---|---|---|
| Base Oil Composition (weight %) | | 88% Group II 12% AE | 76% Group II 24%AE |
| KV40, mm²/s (cSt) | IP71 | | 162.4 |
| KV100, mm²/s (cSt) | IP71 | 12.3 | 14.43 |
| VI | IP226 | 92 | 85 |
| Density, g/cm³ | IP365 | 0.8870 | 0.9005 |
| Flash point (PMCC), °C | IP34 | 238.3 | 236.1 |
| Flash point (COC), °C | IP36 | 254 | 264 |
| Pour point, °C | IP15 | -15 | -12 |
| Colour | ASTM D1500 | 6.1 | >8 |
| TAN, mg KOH/g | IP1A | <0.05 | <0.05 |
| TBN, mg KOH/g | IP276 | 0.22 | 0.47 |
| Sulphur, wt. % | ASTM D4951 | 0.49 | 0.98 |
| Nitrogen, wt. % | ASTM D5762 | 0.019 | 0.032 |
| Demulsibility, secs | IP19 | 405 | 630 |
| Dialysis, % wt | BAM72 | <0.1 | <0.1 |
| Oxidation IP48 | IP48 | | |
| Viscosity ratio | | 1.18 | 1.40 |
| Carbon before, wt. % | | 0.31 | 0.69 |
| Carbon after, wt. % | | 0.87 | 2.37 |
| Carbon, Δ | | 0.56 | 1.68 |
| Carbon types wt % | BAM76 | | |
| Carbon, aromatic C_{A} | | 4.4 | 7.1 |
| Carbon, naphthenic C_{N} | | 63.7 | 63.0 |
| Carbon, paraffinic C_{P} | | 31.9 | 29.9 |
| Viscosity gravity constant | ASTM D2501 | 0.799 | 0.902 |

Further base oils were prepared using the Group II base stock and the aromatic extract in other amounts. Oxidation properties of the base oils were tested according to the Institute of Petroleum procedure IP48 and the results are given in Table V below :

**Table V.**

| Wt. % aromatic extract in base oil | Sample | Δ viscosity Ratio | Carbon unoxidized % | Carbon oxidized % | Δ carbon % |
|---|---|---|---|---|---|
| 0 | Experiment A | 3.06 | 0.05 | 0.60 | 0.55 |
| 3 | Example 3 | 1.18 | 0.12 | 0.33 | 0.21 |
| 6 | Example 4 | 1.11 | 0.20 | 0.37 | 0.17 |
| 12 | Example 1 | 1.18 | 0.31 | 0.87 | 0.56 |
| 18 | Example 5 | 1.30 | 0.52 | 1.35 | 0.83 |
| 24 | Example 2 | 1.40 | 0.69 | 2.37 | 1.68 |
| 30 | Example 6 | 1.60 | 0.87 | 2.76 | 1.89 |

Experiment A is not according to the present invention because it does not contain any aromatic extract.

The results of the change in carbon (Δ carbon) and viscosity ratio at the different concentrations of aromatic extract in the base oil are also shown in Figure 1.

The results of the Δ carbon and viscosity ratio show that the aromatic extract provides an improvement in Δ carbon at a concentration of aromatic extract up to about 12 % by weight and an improvement in viscosity ratio at a concentration of aromatics extract of up to 30 % by weight.

These results show the beneficial effect of the presence of 0.2 to 30 % by weight of aromatic extract in a base oil composition comprising a base stock comprising at least 95 weight % saturated hydrocarbons.

Lubricant compositions suitable for use in a marine 4-stroke engine using heavy fuel were prepared using a salicylate-rich additive package and base oils comprising different amounts of aromatic extract.

Properties of the formulated lubricant compositions are shown in Table VI below.

**Table VI.**

| Base oil blend used in lubricant | Test Methods | 100% Group II | 88% Group II 12% AE | 76% Group II 24% AE |
|---|---|---|---|---|
| Sample | | | Example 7 | Example 8 |
| KV40, mm²/s (cSt) | IP71 | 99.28 | 124.2 | 160.4 |
| KV100, mm²/s (cSt) | IP71 | 11.63 | 13.12 | 15.04 |
| VI | IP226 | 105 | 99 | 93 |
| TBN, mg KOH/g | IP276 | 38.71 | 40.59 | 40.29 |
| Pour Point, °C | IP15 | -21 | -18 | -15 |
| Flash point (PMCC), °C | IP34 | 218.8 | 220.2 | 226.2 |
| Metals, ppm | ICP | | | |
| Ca | | 14996 | 13641 | 13667 |
| P | | 565 | 481 | 483 |
| Zn | | 518 | 505 | 503 |
| Si | | 8 | 11 | 12 |
| Na | | 54 | 50 | 50 |
| Foam, ml/ml | IP146 | | | |
| Sequence 1 | | 0/0 | 0/0 | 0/0 |
| Sequence 2 | | 280/0 | 350/0 | 390/0 |
| Sequence 3 | | 0/0 | 10/0 | 10/0 |
| Density, g/cm³ | IP365 | 0.9018 | 0.9123 | 0.9231 |
| ARV, mins | IP313 | 20.6 | 25.1 | 31.7 |
| Demulsibility, ml | ASTM D1401 | 1/0/79 (60 mins. 82 °C) | 1/0/79 (60 mins. 82 °C) | 1/0/79 (60 mins. 82 °C) |

Oxidation properties of the lubricant compositions were measured. The results are shown in Table VII below.

**Table VII.**

| Base oil used in lubricant composition | Test Method | 100% Group II | 88% Group II 12% AE | 76% Group II 24% AE |
|---|---|---|---|---|
| Sample | | | Example 7 | Example 8 |
| Isothermal oxidation test (ISOT) | ISOT 72hrs @ 165°C | | | |
| Δ BN, % | | -1.42 | -2.60 | -2.87 |
| Δ KV 40, % | | +3.02 | +8.9 | +22.8 |
| Δ KV100, % | | +0.25 | +0.70 | +1.47 |
| Panel Coker aluminium panels 22hrs 325°C | BEM144 | 68.1 | 121.4 | 137.1 |
| Panel Coker Steel panels 2x4hrs 320°C Average | In-house method | 107.4/147.7 | 33.3/28.9 | 10.2/9.4 |
| | | 127.6 | 31.1 | 9.8 |
| Cu corrosion 3 hrs 120°C | ASTM D130 | N/A | 1a slight tarnish | 1a slight tarnish |
| Cu corrosion 3hrs 150°C | ASTM D130 | N/A | 1a slight tarnish | 1a slight tarnish |
| Rusting characteristics | IP135B | N/A | No rusting | No rusting |

The results in Table VII show some improvement is observed within the Panel Coker Test using steel panels undertaken according to the in-house method at 12 and 24 % by weight aromatic extract indicating an improvement within the solvency of the lubricant composition when aromatic extract is used.

Wear properties of the lubricant compositions were measured using a Cameron Plint test. The results are shown in Table VIII below.

**Table VIII.**

| | Test | Wear vol. mm³ | Specific Wear Rate (SWR) m³/Nm | Mean Wear Scar Depth (MWSD) µm | Pin wear mm |
|---|---|---|---|---|---|
| Bad reference | 1074 | 0.0643 | 5.82 E-17 | 22.7 | 0.024 |
| Good reference | 1082 | 0.0119 | 7.35 E-18 | 12.1 | 0.006 |
| 100% Gp II | 006A/02 | 0.00182 | 1.12 E-18 | 18.9 | 0.007 |
| 88% Group II 12% AE | 010A/01 | 0 | 0.00 E+00 | 0 | 0.002 |
| 76% Group II 24% AE | 011A/01 | 0.0254 | 1.57 E-17 | 18 | 0.009 |

The wear properties were compared against reference lubricant formulations with good and bad wear performance. The results show an exceptionally good wear performance for a lubricant composition with a base oil comprising 12 % by weight aromatic extract. However, at the higher concentration of 24 % by weight aromatics extract in the base oil, there is no significant improvement in wear performance compared to the composition with 100% Group II base oil. This data implies that there is an optimum concentration of aromatic extract for wear performance.

## Claims

1. A method of making a liquid marine lubricant base oil composition which method comprises blending:
(i) a base stock comprising at least 95 % by weight saturated hydrocarbons, the base stock comprising a hydroprocessed base stock and/or a base stock derived from Fischer-Tropsch synthesised, waxy, paraffinic hydrocarbon material, with
(ii) 0.2 to 30% by weight of an aromatic extract which has an aromatics content of 60 to 85% by weight as measured by ASTM D 2007 and a dimethyl sulphoxide extractable polycyclic aromatics content of less than 3 weight % as measured by IP 346,
to make a liquid lubricant base oil composition.

2. The use of 0.2 to 30 % by weight of an aromatic extract which has an aromatics content of 60 to 85% by weight as measured by ASTM D 2007 and a dimethyl sulphoxide extractable polycyclic aromatics content of less than 3 weight % as measured by IP 346 in a liquid marine lubricant base oil composition which base oil comprises a base stock comprising at least 95 % by weight saturated hydrocarbons, which hydrocarbons comprise a hydroprocessed base stock and/or a base stock derived from Fischer-Tropsch synthesised, waxy, paraffinic hydrocarbon material, to mitigate at least one of the deficiencies of the base stock selected from the group consisting of poor dispersancy, poor seal swell performance, poor solubility of additives and low compatibility with fuel oil in marine engine applications.

## Patentansprüche

1. Verfahren zur Herstellung einer flüssigen Schiffs-Schmierstoffbasisölzusammensetzung, wobei das Verfahren das Mischen:
(i) eines Grundöls, umfassend mindestens 95 Gew.-% gesättigter Kohlenwasserstoffe, wobei das Grundöl ein hydroprozessiertes Grundöl und/oder ein Grundöl, gewonnen aus einem durch Fischer-Tropsch synthetisierten, wachsartigen, paraffinischen Kohlenwasserstoffmaterial, ist, mit
(ii) 0,2 bis 30 Gew.-% eines aromatischen Extrakts, der einen Aromatengehalt von 60 bis 85 Gew.-%, gemessen nach ASTM D 2007, und einen Gehalt an Dimethylsulfoxid-extrahierbaren, polycyclischen Aromaten von weniger als 3 Gew.-%, gemessen nach IP 346, hat,
unter Herstellung einer flüssigen Schmierstoffbasisölzusammensetzung umfasst.

2. Verwendung von 0,2 bis 30 Gew.-% eines aromatischen Extrakts, der einen Aromatengehalt von 60 bis 85 Gew.-%, gemessen nach ASTM D 2007, und einen Gehalt an Dimethylsulfoxid-extrahierbaren, polycyclischen Aromaten von weniger als 3 Gew.-%, gemessen nach IP 346, hat, in einer flüssigen Schmierstoffbasisölzusammensetzung, wobei das Basisöl ein Grundöl, umfassend mindestens 95 Gew.-% gesättigter Kohlenwasserstoffe, umfasst, wobei die Kohlenwasserstoffe ein hydroprozessiertes Grundöl und/oder ein Grundöl, gewonnen aus einem durch Fischer-Tropsch synthetisierten, wachsartigen, paraffinischen Kohlenwasserstoffmaterial, umfassen, zur Minderung zumindest eines der Mängel des Grundöls, ausgewählt aus der Gruppe, bestehend aus schlechtem Dispergiervermögen, schlechtem Dichtungsquellverhalten, schlechter Löslichkeit von Additiven und geringer Kompatibilität mit Brennstofföl in Schiffsmotorenanwendungen.

## Revendications

1. Procédé pour préparer une composition d'huile de base lubrifiante marine liquide, lequel procédé comprend le mélange
(i) d'une huile de base comprenant au moins 95 % en poids d'hydrocarbures saturés, l'huile de base comprenant une huile de base hydrotraitée et/ou une huile de base dérivée d'un matériau hydrocarboné paraffinique cireux synthétisé par le procédé Fischer-Tropsch, avec
(ii) 0,2 à 30 % en poids d'un extrait aromatique qui a une teneur en aromatiques de 60 à 85 % en poids, telle que mesurée conformément à la norme ASTM D2007, et une teneur en aromatiques polycycliques extractibles au diméthylsulfoxyde inférieure à 3 % en poids, telle que mesurée conformément à la norme IP 346,
pour préparer une composition d'huile de base lubrifiante liquide.

2. Utilisation de 0,2 à 30 % en poids d'un extrait aromatique qui a une teneur en aromatiques de 60 à 85 % en poids, telle que mesurée conformément à la norme ASTM D2007, et une teneur en aromatiques polycycliques extractibles au diméthylsulfoxyde inférieure à 3 % en poids, telle que mesurée conformément à la norme IP 346, dans une composition d'huile de base lubrifiante marine liquide qui comprend une huile de base comprenant au moins 95 % en poids d'hydrocarbures saturés, lesquels hydrocarbures comprennent une huile de base hydrotraitée et/ou une huile de base dérivée d'un matériau hydrocarboné paraffinique cireux synthétisé par le procédé Fischer-Tropsch, pour réduire au moins l'une des insuffisances de l'huile de base choisies dans le groupe constitué par un médiocre pouvoir dispersant, une médiocre performance de gonflement des joints, une médiocre solubilité des additifs et une faible compatibilité avec le gazole dans des applications à des moteurs marins.
